

3,494,841

**PROCESS OF SELECTIVE FLUORINE REMOVAL  
FROM ZINC CONCENTRATES AND MANGANESE DIOXIDE**

Bruno Orlandini and Walter Schmittroth, Kellogg, Idaho, assignors, by mesne assignments, to The Bunker Hill Company, Kellogg, Idaho, a corporation of Delaware  
No Drawing. Filed Sept. 25, 1967, Ser. No. 670,441  
Int. Cl. C22d 1/22

U.S. Cl. 204—119

7 Claims

10

**ABSTRACT OF THE DISCLOSURE**

To prevent fluorine etching of the aluminum oxide coated cathode during the electrolytic deposition of zinc, the zinc concentrate is pre-leached before the roasting process to remove acid soluble fluorine compounds from the concentrate. The zinc concentrate is pre-leached utilizing a weak acid solution of sulfuric acid having a concentration of 1% to 5% sulfuric acid by weight. The manganese dioxide additive may also be pre-leached by the same process to remove acid soluble fluorine compounds before the manganese dioxide is added to the calcine leach pulp.

**DESCRIPTION OF THE INVENTION**

This invention relates to the electrolytic process for recovering zinc and more particularly to processes for preventing fluorine from etching the aluminum cathodes as the zinc is being deposited thereon in the electrolytic bath.

To properly understand and appreciate this invention it is necessary to be familiar with the general electrolytic process for recovering metallic zinc having a purity of greater than 99.99% from zinc ore.

The zinc is generally mined from the earth as a zinc sulfide. The zinc sulfide ore is often referred to as zinc blend. After crushing, the ore is concentrated by flotation. A host of other materials of various concentrations besides zinc sulfide is included in the concentrate depending upon the source of the ore. Iron compounds are generally included in the concentrate. Often the concentrate contains fluorine compounds in concentration of more than 3 milligrams per hundred grams of concentrate. Although the zinc sulfide is somewhat soluble in relatively strong acid, it has been found that by roasting the concentrate, the zinc sulfide is transferred into a more soluble compound of zinc oxide. The roasted zinc concentrate is referred to as zinc calcine. The calcine is then leached in a sulfuric acid solution to separate those impurities that are soluble in the electrolyte from those materials that are insoluble in the electrolyte. Zinc oxide and some impurities dissolve in the sulfuric acid leach. Included in the soluble impurities are generally small amounts of metallic compounds of iron, cobalt, arsenic, antimony, nickel, etc. Fluorine compounds such as sodium fluoride and calcium fluoride also dissolve in the leach.

If the amounts of the dissolved metallic impurities are greater than desired, various additives are added to precipitate the metallic impurities from the solution before the solution passes to the electrolytic cell. Generally manganese dioxide is added to oxidize the iron to the ferric state which in turn precipitates out as ferric compounds. Frequently the manganese dioxide additive contains fluorine compounds. The leach pulp is then filtered to remove the precipitate. Metallic zinc is then added to the leach filtrate to precipitate many of the metallic impurities such as copper, cobalt, nickel, etc. The leach filtrate is again filtered to remove the precipitates. The concentrated zinc solution is then carried to the electrolytic cell where an electrical force is applied between the cathode and anode

causing the zinc ions to migrate and deposit upon a cathode.

The cathodes are generally made of metallic aluminum with a coating of aluminum oxide formed on the surface thereof to act as a barrier to prevent the zinc from bonding to the metallic aluminum. However, if the electrolyte contains fluorine, the fluorine etches away the aluminum oxide protective barrier enabling the zinc to bond directly to the metallic aluminum. Such a metallic bond makes it almost impossible to physically remove (strip) the zinc from the cathode without damaging the cathode or re-dissolving the zinc. As a practical matter, if a metal to metal bond occurs, substantial additional costs are incurred to remove the zinc from the cathode.

Several attempts have been made to minimize the fluorine etching of the cathodes. One method used, is to bleed the electrolyte from the electrolytic cell when the fluorine concentration in the electrolyte exceeds a certain value. The electrolyte bled from the cell contains a substantial amount of valuable zinc and acid which represents lost production or requires costly further processing to remove the fluorine and recycling the zinc solution back to the electrolytic cell.

Another method used to minimize the fluorine etching of the cathode while the zinc is being deposited on the cathode is to let the zinc solution sit in the cell with the cathode immersed therein for about 15 minutes before the electrical force is applied between cathode and anode. During this interval the surface of the aluminum oxidizes to form a reinforced protective barrier. Such a method substantially reduces the efficiency of the electrolytic process, because 15 minutes of each bath cycle is unproductive and may be considered down time necessitating additional labor to energize the cell.

One of the principal objects of this invention is to provide a vastly improved method of preventing the fluorine etching of the cathode.

An additional object of this invention is to remove the fluorine compounds that are soluble in the electrolyte before the constituents are added to the electrolytic cell.

A further object of this invention is to provide a pre-leaching process for removing electrolyte soluble fluorine compounds from the zinc concentrate and the manganese dioxide before they are added to the electrolytic cell.

An additional object of this invention is to pre-leach the electrolyte soluble fluorine compounds from the zinc concentrate before the zinc concentrate is roasted.

This invention involves the removal of the electrolyte soluble fluorine compounds from the principal sources—the zinc concentrate and the manganese dioxide additive.

With respect to the zinc concentrate, the electrolyte soluble fluorine compounds are removed therefrom prior to roasting. It has been found that by contacting the zinc concentrate (zinc sulfide) with a weak sulfuric acid solution (pre-leaching) that the electrolyte soluble fluorine compounds will dissolve without dissolving appreciable amounts of the zinc sulfide. It has been found that a weak sulfuric acid leach solution of between 1% and 5% sulfuric acid by weight is particularly effective in dissolving the soluble fluorine compounds without dissolving an appreciable amount of zinc sulfide.

In performing the pre-leaching process the following preferred procedure was found to be particularly effective. The zinc concentrate was mixed with water to form a slurry in the proportions of 100 grams of zinc concentrate per 250 milliliters of slurry. The 250 milliliters of slurry was mixed with an equal amount of a weak acid solution. The weak acid solution was formulated by adding between 20 and 100 grams of sulfuric acid per liter of water. The weak acid solution and the slurry were agitated to increase the rate of dissolution of the soluble fluorine compounds.

At temperatures between 20-40° C. it has been found that four hours of agitation was sufficient.

After the leach pulp is agitated the solution containing the dissolved fluorine is filtered from the zinc concentrate. Utilizing this procedure it was found that the soluble fluorine concentration in the zinc concentrate could be readily and effectively reduced well below 3 milligrams per 100 grams of zinc concentrate. The zinc concentration is then roasted to form the zinc oxide. In this manner the electrolyte soluble fluorine compounds are removed from the zinc concentrate to prevent the soluble fluorine compounds from being carried to the electrolytic cell.

This pre-leaching process has been utilized on zinc concentrate batches from many parts of the world. The pre-leaching of zinc concentrate A with a 1% sulfuric acid solution removed 21.2 milligrams of fluorine and 0.31 gram of zinc per 100 grams of zinc concentrate. Utilizing a 5% sulfuric acid solution, 24.1 milligrams of fluorine and 1.06 grams of zinc per 100 grams of concentrate were pre-leached from the zinc concentrate to reduce the fluorine content well below the maximum allowable of 3 milligrams of fluorine per 100 grams of zinc concentrate.

The pre-leaching of zinc concentrate B with a 1% sulfuric acid solution removed 7.6 milligrams of fluorine and 0.20 gram of zinc per 100 grams of zinc concentrate. Utilizing a 5% pre-leaching sulfuric acid solution with the zinc concentrate B, 25.0 milligrams of fluorine and 0.64 gram of zinc per 100 grams of zinc concentrate were removed reducing the fluorine concentration well below the maximum allowable. With respect to zinc concentrate C which came from an area having a very large concentration of acid soluble fluorine compounds in the ore, 353 milligrams of fluorine and 1.06 grams of zinc were removed from the concentrate utilizing a 5% weak acid leach solution.

In like manner the electrolyte soluble fluorine compounds may be pre-leached from the manganese dioxide additive so that soluble fluorine compounds do not enter the electrolyte when the manganese dioxide is added during the leaching step of the process.

It should be understood that various other preferred embodiments may readily be devised by those skilled in the art that incorporate the principles of the invention and fall within the scope thereof. Therefore, only the following claims are intended to define this invention.

What is claimed is:

1. In a process for recovering metallic zinc from ore containing fluorine compounds by separating the ore to form a zinc concentrate, roasting the zinc concentrate to form zinc calcine, dissolving the calcine in a sulfuric acid solution to form a zinc electrolyte and separating the zinc from the electrolyte by electrolysis utilizing a cathode having an aluminum oxide coating that is susceptible to fluoride etching, the improvement in which the process includes a pre-leaching sub-process of removing the aque-

ous or acid soluble fluorine compounds from the zinc concentrate prior to roasting by contacting the zinc concentrate with a weak acid leach solution having a sulfuric acid concentration which is sufficient to dissolve the soluble fluorine compounds without dissolving appreciable amounts of the zinc concentrate.

2. The process as defined in claim 1 wherein the pre-leaching sub-process is performed with a leach solution containing between 1% and 5% sulfuric acid by weight.

3. The process as defined in claim 1 wherein the pre-leaching sub-process includes the addition of water to the zinc concentrate to form a slurry prior to mixing with the weak acid solution.

4. The process as defined in claim 3 wherein the water and zinc concentrate are mixed to form a slurry in proportion having 100 grams of zinc concentrate per 250 milliliter and wherein the slurry is mixed with an equal amount of weak acid solution having between 20 and 100 grams of sulfuric acid per liter of solution.

5. The process as defined in claim 4 wherein the resultant slurry acid solution is agitated to increase the dissolution of the soluble fluorine compounds.

6. In a process for recovering metallic zinc from ores containing iron compounds by separating the ore to form a zinc concentrate, roasting the zinc concentrate to form zinc calcine, dissolving the calcine in a sulfuric acid solution to form a zinc leach pulp, adding manganese dioxide to the leach pulp to oxidize and precipitate the iron, separating the precipitate from the pulp to form a zinc solution and separating the zinc from the solution by electrolysis utilizing a cathode having an aluminum oxide coating that is susceptible to fluorine etching, the improvement in which impure manganese dioxide is pre-leached prior to adding to the leach pulp to remove soluble fluorine compounds from the manganese dioxide to prevent the fluorine etching of the cathode, said pre-leaching being performed by contacting the impure manganese dioxide with a weak acid leach solution that has a sulfuric acid concentration which is sufficient to dissolve the soluble fluorine compounds without dissolving appreciable amounts of manganese dioxide.

7. The process as defined in claim 6 wherein the manganese dioxide concentrate is pre-leached with a leach solution containing between 1% and 5% sulfuric acid by weight.

#### References Cited

##### UNITED STATES PATENTS

|           |        |            |       |         |
|-----------|--------|------------|-------|---------|
| 1,542,935 | 6/1925 | Greenawalt | ----- | 204—119 |
| 629,686   | 7/1899 | Hoepfner   | ----- | 204—118 |

JOHN H. MACK, Primary Examiner

R. L. ANDREWS, Assistant Examiner

U.S. CL. X.R.

204—118